

July 7, 1925.

**1,545,305**

F. M. CRAPO ET AL

## METAL TREATING APPARATUS AND PROCESS

Filed April 21, 1924



Patented July 7, 1925.

## UNITED STATES PATENT OFFICE.

FREDERICK M. CRAPO AND WILLIAM BAYLIS, OF MUNCIE, INDIANA.

## METAL-TREATING APPARATUS AND PROCESS.

Application filed April 21, 1924. Serial No. 707,863.

*To all whom it may concern:*

Be it known that we, FREDERICK M. CRAPO and WILLIAM BAYLIS, citizens of the United States, residing at Muncie, in the county of Delaware and State of Indiana, have invented a new and useful Metal-Treating Apparatus and Process, of which the following is a specification.

Our invention relates to an improved process and apparatus for chemically heat-treating iron and steel articles, especially wire or rod. More specifically, this process and apparatus is for use in making the protected metal set forth in the co-pending application of Frederick M. Crapo, Serial No. 679,650, filed December 10, 1923, now Patent No. 1,501,887, granted July 15, 1924.

According to such prior application, considered very briefly and very specifically, iron or low-carbon steel wire which is subsequently to be zinc-coated is chemically heat-treated by being passed through a bath of molten surface-hardening treating material in which the chemical heat-treatment is effected. By such chemical heat-treatment, there is produced in the wire a permeative addition by chemical change and a heat-treatment; and in the specific process there set forth these include annealing and surface hardening. The treating material used with best success contained carbonizing material, such as commercial cyanide mixtures.

It is found, however, that the molten salts containing cyanide adversely affect any ordinary container therefor, and make the life of such container very short; and also that a considerable volume of such molten salts must be used, that there is a considerable loss of salts in operation, and that replenishment of the salt bath must be made with a salt mixture of rather high cyanide content, when the container directly holds the salts.

It is the fundamental object of our present invention to reduce or eliminate this injurious effect on the container, to reduce the volume of salts, to reduce the loss of salts, and to make it possible to replenish the salt bath with a salt mixture of lower cyanide content.

In carrying out our invention, we float the surface-hardening treating material to be used in the chemical heat-treatment on a heavier molten material, conveniently

lead, which lead in turn is carried in the container. The treating material is confined to a definite part of the surface of the heavier molten material, by a suitable circumscribing band or ring supported so that its walls extend both above and below such surface. Thus the treating material is kept from contact with the container, and adverse effects thereof on the container proper are eliminated. The band itself may be adversely affected by the treating material, but this effect on the band is much less harmful because the band is not subjected to the flames as the container is, and in any case the band can be replaced at relatively small cost, inconvenience, and delay, as compared with the container.

The articles to be treated, such as the iron or steel wire, are chemically treated in the treating material in the band. This treating material conveniently consists of molten salts, and we find commercial cyanide mixtures to be very advantageous. This treatment is most conveniently obtained, with economy in the use of salts, if the wire is first passed into the molten lead at a point outside of the band, and carried along beneath the surface of the molten lead to a point beneath the band, then passed upward through the molten salts, and thence carried to any desired subsequent treatments. While passing through the molten lead, the wire is heated so that the time it need remain in the salts may be even shorter than that contemplated in the aforesaid Crapo application. The wire is well annealed as it leaves the molten salts; and, further, carries with it a slight film of such salts, which film probably continues its action on the surface of the wire for an appreciable time as the wire cools and in addition prevents oxidation of the surface of the wire. This whole operation is continuous in the case of wire and rods.

After this chemical heat-treatment, the wire may be passed through a suitable bath or baths, such as a water bath to remove the adhering salts and a fluxing bath; and then is zinc-coated, as by being passed through a bath of molten zinc, if that is desirable. This zinc coating is of the superior quality of the Crapo product set forth in the aforesaid prior application.

The accompanying drawing illustrates our invention: Fig. 1 is a longitudinal sectional

view showing diagrammatically an apparatus embodying our invention as used for chemically heat-treating wire just prior to zinc-coating; Fig. 2 is a longitudinal sectional view showing diagrammatically an apparatus embodying our invention as used for chemically heat-treating rods before drawing, or wire at an intermediate stage of drawing; Fig. 3 is an enlarged transverse section on the line 3—3 of Figs. 1 and 2; and Fig. 4 is a fragmental plan showing the salt-confining band.

The iron-vase wire 10 is presumed to have been passed previously through the desired sizing dies, until it has reached the gage at which it is desired to zinc-coat it. Then it is passed into a container 11, containing molten lead 12; the lead being maintained molten by a suitable fire 13 beneath such container. The wire is passed for some distance through the lead, beneath its surface, and is then passed up through a bath of molten salts 14 floated on top of the molten lead and heated therefrom. The salts 14 may also be heated from above, as by an auxiliary gas burner 15; but the lead is desirably maintained at higher temperature than the salts, so that wire or rod entering the salts from below will be hotter than such salts. The salts are confined to a definite part of the surface of the lead by a circumscribing band or ring 16. The wire after it leaves the molten salts is passed through any suitable baths, of which we have shown a bath 17 of water for removing any adhering salts and a bath 18 of a suitable flux such as hydrochloric acid or zinc chloride; then if desired over a hot plate 19 to insure drying of the wire; and then through a bath 20 of molten zinc in which the wire takes its zinc coating. From the zinc-coating bath 20, of molten zinc, the wire passes to the winding reel 21. All this is in a continuous process, with the wire moving continuously in the direction of the arrows. The intermediate baths shown, such as the water bath 17 and the fluxing bath 18, are merely to exemplify any intermediate treatments which it may be desired to give the wire, and are not limitations on what such treatments may be. Further, the zinc-coating may be applied in various ways; although the way we prefer to apply it, especially to wire, is by passing the wire through a bath of molten zinc. Such zinc-coating bath is advantageously maintained at about 840° to 900° F., in any convenient way, though that temperature may be varied in the judgment of the operator.

The band or ring 16 may be of any desired size and shape, to permit any desired number of wires to pass through it, and may be supported in any suitable way. It is shown as rectangular, supported by laterally projecting arms 22, which project over

and are bolted to the sides of the container 11. The walls of the band 16 project downward slightly into the molten lead, and upward above the upper surface of the molten salts contained within it. These salts are maintained at a temperature somewhat above their melting point, advantageously between 1200° and 1350° F., by heat from the bath of molten lead below, and from the auxiliary burner 15 if that is used, and from the wires passing through the salts. The lead is desirably maintained between 1275° to 1375° F. It is usually desirable that the lead be covered with a pulverized hard coal or charcoal layer 23, which serves both to prevent heat loss by radiation and to lessen oxidation of the lead. For carrying off fumes, a hood 24 may be provided over the bath 11. The passage of the wire through the bath 11 is guided by suitable sinkers 25 and 26, of which the latter may conveniently be formed on a lower edge of the band 16, as shown in Figs. 1 and 2, although as shown in Fig. 4 the band 16 may be made without having such sinker 26 formed thereon. The band 16 is desirably covered by removable cover plates 27, to lessen cooling of the salts. A pin-board wipe 28 is desirably provided for the wires as they emerge from the salts. This pin-board wipe comprises a cross-bar over which the wires slide, and a series of pins projecting from said cross-bar between said wires to keep them separated.

The wire as it passes through the molten lead and the molten salts is given the desired chemical heat-treatment. The wire is annealed and pre-heated in its passage through the molten lead. Then, as the wire passes up from the molten lead into and through the molten salts, it receives a surface-hardening treatment. The salts we prefer to use contain some cyanide, and we find that a cyanide mixture containing one part sodium cyanide, two parts sodium chloride, and four parts sodium carbonate produces good results. This produces on the wire a very thin surface change, probably involving carbonization and other things; and in addition the wire as it passes through the lead and through the salts is thoroughly and effectively annealed.

Referring now to the apparatus shown in Fig. 2:

Here the tank 11, lead 12, fire 13, molten salts 14, and circumscribing band 16 are substantially the same as illustrated in Fig. 1. The wire or rod 10', however, is assumed not to have reached the final gage, and may be merely the rod before there has been any drawing operation. Such rod as it passes through the lead and salts is chemically heat-treated. After the rod or wire 10' passes from the molten salts, it may pass through a suitable water bath 17, to remove any ad-

hering salts, and may then be wound on a winding reel 21 ready for subsequent drawing.

The amount of salts necessary with the band 16 is very much less than is necessary if such salts comprise the entire contents of the container 11. This reduces the loss of salts in operation, largely because of the reduction in exposed area of such salts.

10 Moreover, because of this reduction in loss of salts and because of the relatively small volume of salts, replenishment of the salts may be made with cyanide mixtures having lower cyanide content, as the quantities used in replenishing are much larger fractions of the whole. Further, the band 16 holds the salts away from the container 11, so that there is no effect produced on such container by the salts. This increases the 20 life of the container many times. The effect of the salts on the band 16 is not of great moment; not only because such band is not exposed to the flame, but also because if the salts in any case do adversely affect the band the latter may be replaced easily and cheaply, which may be done without any loss of material, and without any danger such as occurs from the burning out of a container, and without the labor 25 which is necessary to set a new container in place in its foundations.

We claim as our invention:—

1. In an apparatus for chemically heat-treating metal articles, the combination of a container holding molten material, a surface-hardening treating material floating on part of the surface of said molten material, and a circumscribing band for confining said treating material to part of said 40 surface and preventing it from coming in contact with said container.

2. The combination set forth in claim 1, with the addition that said treating material contains cyanide.

45 3. The combination set forth in claim 1, with the addition of means for heating said treating material from above.

4. The combination set forth in claim 1, with the addition that said molten material 50 is lead.

5. The combination set forth in claim 1, with the addition that said molten material is lead, and that said treating material contains cyanide.

55 6. The combination set forth in claim 1, with the addition that said treating material is in a molten state but at a lower temperature than that of the body of molten material on which it floats.

60 7. The combination set forth in claim 1, with the addition of means for conducting a wire or rod through said two materials in series.

8. The combination set forth in claim 1, with the addition of means for conducting a

wire or rod into said molten material outside of said band and then through the treating material inside of said band.

9. The combination set forth in claim 1, with the addition of means for passing a 70 wire or rod down into and then up out of said molten material, one of said passings being inside of and one outside of said band.

10. The combination set forth in claim 1, 75 with the addition of means for passing a wire or rod down into and then up out of said molten material, one of said passings being inside of said band.

11. The combination set forth in claim 1, 80 with the addition of means for passing a wire or rod through the treating material within said band.

12. The combination set forth in claim 1, 85 with the addition of means for supporting said band from said container.

13. The process of chemically heat-treating iron or steel articles, comprising floating a surface-hardening treating material on the surface of a bath of molten material in 90 a container, confining such treating material to part of such surface and out of contact with the container, and passing such articles through said treating material.

14. The process of chemically heat-treat- 95 ing iron or steel articles, comprising floating a surface-hardening treating material on the surface of a bath of molten material in a container, confining such treating material to part of such surface and out of contact 100 with the container, and passing such articles through said treating material and said molten material in series.

15. The continuous process of chemically heat-treating iron or steel wire or rod, comprising floating a surface-hardening treat- 105 ing material on the surface of a bath of molten material in a container, confining such treating material to part of such surface and out of contact with the container, and continuously passing such wire or rod 110 through said treating material.

16. The continuous process of chemically heat-treating iron or steel wire or rod, comprising floating a surface-hardening treat- 115 ing material on the surface of a bath of molten material in a container, confining such treating material to part of such surface and out of contact with the container, and continuously passing such wire or rod 120 through said treating material and said molten material in series.

17. The process of chemically heat-treat- 125 ing iron or steel articles, comprising floating a surface-hardening treating material on the surface of a bath of molten lead in a container, confining such treating material to a part of such surface and out of contact with the container, and passing such articles through said treating material. 130

18. The process of chemically heat-treating iron or steel articles, comprising floating a surface-hardening treating material containing cyanide on the surface of a bath of molten material in a container, confining such treating material to part of such surface and out of contact with the container, and passing such articles through said treating material.
19. The process of chemically heat-treating iron or steel articles, comprising floating a surface-hardening treating material containing cyanide on the surface of a bath of molten lead in a container, confining such treating material to part of such surface and out of contact with the container, and passing such articles through said treating material.
20. The process of chemically heat-treating iron or steel articles, comprising floating a surface-hardening treating material containing cyanide on the surface of a bath of molten material in a container, confining such treating material to part of such surface, and passing such articles through said treating material.
21. In an apparatus for chemically heat-treating metal articles, the combination of a container holding molten material, a surface-hardening treating material floating on part of the surface of said molten material, and means for confining said treating material to part of said surface.

In witness whereof, we have hereunto set our hands at Muncie, Indiana, this 15th day of April, A. D. one thousand nine hundred and twenty-four.

FREDERICK M. CRAPO.  
WILLIAM BAYLIS.